

Oct. 25, 1932.

A. KAZENMAIER ET AL

1,883,932

ELECTRIC CONDENSER

Filed July 28, 1927



Inventors  
August Kazenmaier  
Walter Dorn  
by Stearns & Kay  
their attorneys

## UNITED STATES PATENT OFFICE

AUGUST KAZENMAIER AND WALTER DORN, OF STUTTGART, GERMANY, ASSIGNEES TO  
ROBERT BOSCH AKTIENGESELLSCHAFT, OF STUTTGART, GERMANY

## ELECTRIC CONDENSER

Application filed July 28, 1927, Serial No. 209,175, and in Germany August 28, 1926.

This invention relates to electric condensers and methods of manufacturing the same and it relates particularly to condensers composed of alternate layers of laminations of conducting material and insulating or dielectric material.

A principal object of the invention is to provide a condenser of the above character with a durable, insulating, protective coating which will cling tenaciously to the condenser and at the same time be impervious to moisture.

Other objects of the invention will be apparent from the following description.

15 It is highly desirable to protect electric condensers of the above mentioned type with a coating of any of the many synthetic resins of the phenol-formaldehyde type, such, for example, as "bakelite" because such substances are hard and impervious to moisture. However, a coating of this material does not adhere well to the metal surfaces of the condensers and furthermore, because of its brittleness, it is easily cracked or broken, so that 25 such a coating is either defective from the start or becomes so after a short time.

It is also desirable to protect such condensers with a coating of shellac or similar gum-lac or resinous substance because shellac adheres well to metal, is a good insulator and is comparatively elastic or non-brittle. However, a shellac coating of condensers is objectionable because it does not resist moisture.

According to the present invention the advantages of the above mentioned substances are combined and a durable, reliable, moisture-proof coating is secured by first coating the condenser with a solution of shellac and thereupon with a solution of a synthetic resin 35 or phenolic condensation product such as "bakelite". In this case, the protective coating of shellac, which adheres well to the metal parts, is in turn protected, especially from moisture, by the layer or coating of "bakelite" or the like. The shellac forms a binder 45 between the layer of "bakelite" or the like and the metal parts.

The accompanying drawing illustrates a condenser embodying our invention. The condenser proper *f* comprises two strips of

thin metal foil and two strips of insulating material rolled up into the form of a roll or cylinder. The four strips are arranged in the manner well known so that the strips of metal alternately are placed back from one edge of the insulating strips and protrude over the other edge of said insulating strips. The protruding strips of metal are then pressed down against the ends of the roll to form metal layers or discs *b* which are insulated from each other by the strips of insulating material. The condenser thus formed is inserted in a metallic casing *a*, in which is inserted an insulating sleeve *d*. One of the strips of metal foil is wound around and thereby connected with an inner metallic cylinder *e*, the lower disc *b* being connected to the casing *a*. This casing is closed by an insulating disc *c* and the assembly thus formed is surrounded with a first coating layer *g* of 70 shellac and a second protecting layer *h* of artificial resin.

The shellac is applied to the condenser in any manner desired, the simplest way being by immersion, particularly if the condenser is to be coated all over. However, the shellac may be applied in other ways, with a brush, for example, particularly if it is only a question of providing the condenser with a protective coating in places. The coating of artificial resin or "bakelite" may be applied in the same manner. Thereupon the condenser is dried by the application of heat.

It is to be understood that the invention is not limited to the specific construction or procedure described above, but that it includes all the modifications and adaptations which fall within the scope of the appended claims.

What is claimed is:

1. A condenser provided with a protective coating on its metal surfaces comprising a thin coating of a non-brittle resinous electrically insulating material and a thin outer coating of a phenolic condensation product on the protective coating. 90

2. A condenser provided with a protective coating on its metal surfaces comprising a coating of shellac and an outer coating of a phenolic condensation product on the protective coating. 95

3. A condenser provided with a protective coating on its metal surfaces comprising a coating of a non-brittle resinous electrically insulating material adhering to the condenser body and an outer coating of a moisture-proof material adhering to said first coating.
4. Electrical apparatus having metal surfaces provided with a moisture-proof coating which clings tenaciously to the metal surfaces,
- 10 said film coating comprising a coating of a non-brittle electrically insulating tenacious material placed directly on said metal surfaces and a film coating of a water-proof material placed directly on said coating of non-brittle material.
- 15 5. A condenser having a metal surface provided with an outer coating layer of moisture proof material and a layer of insulating non-brittle resinous material between the metal surface and the outer layer, and adhering to the metal surface and to the outer coating layer, and thereby forming a binder between them.
- 20 6. A condenser having a metal surface provided with an outer coating layer of a phenolic condensation product in combination with an intermediate binding layer of shellac between the metal surface and the outer layer, and adhering to both.

30 In testimony whereof we have hereunto affixed our signatures.

AUGUST KAZENMAIER.  
WALTER DORN.

40

45

50

55

60

65